

## UNITED STATES PATENT OFFICE

1,954,026

## SOUND RECORD

George Schneider, Montclair, N. J., assignor to  
Celanese Corporation of America, a corpora-  
tion of Delaware

No Drawing. Application November 7, 1930  
Serial No. 494,205

3 Claims. (Cl. 154—43)

This invention relates to records for reproducing and/or recording sound and relates more particularly to such sound records wherein the sound track is contained in a surface made of a plastic composition containing a derivative of cellulose.

An object of my invention is to prepare sound records from which tones of pure quality may be reproduced and which are relatively inexpensive. 10 A further object of my invention is to prepare sound records having a sound reproducing surface made of a plastic composition containing a derivative of cellulose while the core thereof is made of a cheap composition. Other objects of 15 this invention will appear from the following detailed description.

It has been proposed to make sound records made of plastic compositions containing derivatives of cellulose. Since such cellulosic plastics are relatively expensive, it would be desirable to 20 replace part thereof with a cheaper material, since from the point of view of sound reproduction, it is not necessary that the interior of the record be made of such cellulosic plastic material.

25 I have found that a composition containing rosin and a plasticizer or softening agent for the rosin is an excellent and cheap material that may be employed as a core upon which sheets of cellulosic material may be laminated. The sheets of cellulosic plastics easily adhere to the rosin composition to form a firm bond.

In accordance with my invention, I prepare sound records, the sound reproducing surface of which is formed of a layer or sheet composed of a plastic composition containing a derivative of cellulose and a suitable plasticizer supported on or laminated with a core made of a composition containing rosin and a plasticizer or softening agent for the rosin.

40 For the reproducing surface, a plastic composition containing a suitable derivative of cellulose such as cellulose nitrate or an organic derivative of cellulose may be employed. Such organic derivative of cellulose may be organic esters of cellulose and cellulose ethers. Examples of 45 organic esters of cellulose are cellulose acetate, cellulose formate, cellulose propionate and cellulose butyrate, while examples of cellulose ethers are ethyl cellulose, methyl cellulose and benzyl cellulose.

The cellulose derivative contained in the reproducing surface is plasticized with a plasticizer or suitable softening agent, examples of which are camphor, xylene monomethyl sulfonamid, diethyl phthalate, dimethyl phthalate, triacetin,

triphenyl phosphate, dibutyl tartrate, diethyl tartrate, dibutyl phthalate, etc., the choice depending on the particular cellulose derivative present. As to the proportions of plasticizer to the derivative of cellulose employed, generally I 60 have found that amounts varying from 35 to 60%, say 40%, of the weight of the derivative of cellulose present, produce excellent results. If the record is to be employed for recording sound, a larger amount of plasticizer is employed to impart the desired degree of softness.

65 The cellulosic plastic material preferably contains no hard filling materials, but the use of such hard filling materials is not excluded. While I prefer to employ little or no filling material at all, if it is desired to reduce the cost of the product, a soft or lubricating filler such as talc, not to exceed 25% of the weight of the cellulosic plastic material, may be employed. The pigment employed should preferably be in finely divided form. To impart color, a suitable dye such as nigrosine may be added.

70 The cellulosic plastic material may be made in any desired manner. I prefer to make a plastic mass by gelatinizing the derivative of cellulose and a plasticizer and any other desired ingredients with a volatile solvent such as acetone, alcohol and/or benzene, working the mass on heated masticating rolls to remove excess solvent, and then forming sheets from the mass. Or 75 films may be cast from solutions of the derivative of cellulose or plasticizer in a volatile solvent upon a smooth surface. The sheets or films so formed may be cut into discs corresponding to the size of the record desired, and these discs 80 may be used for laminating with the cores containing the rosin and plasticizer.

85 If desired the plastic composition containing an organic derivative of cellulose may be made in the form of powder by finely dividing the plastic material by gelatinization of the ingredients by a solvent and removing the solvent, or such powder may be formed by finely grinding the dried organic derivative of cellulose and the plasticizer with or without other ingredients. These powders may be molded under heat and pressure around the core piece containing the rosin between the sound matrices to produce the sound record. Alternatively, a coating composition containing the derivative of cellulose and the plasticizer and a volatile solvent may be coated upon the core containing the rosin.

90 As stated, in order to reduce the cost of manufacture, the interiors or cores of the sound records are made of a composition containing a 95 100 105 110

rosin and a plasticizer or softening agent for the rosin. The plasticizer or softening agent is preferably the same one as that employed in the cellulosic plastic composition but it may be other materials such as acetanilid. Further to reduce the cost of the core material, filling materials such as carbon black, iron oxide, silica, barytes, china clay, talc, cotton flock, etc. may be incorporated. If desired shellac or other resins or gums may also be added as may also be dyes like nigrosine.

If a single record is to be made, one film or sheet of cellulosic plastic is applied to one side of the core containing the rosin; if a double record is to be made a sheet or film is applied to each side of the core.

In making the core material, the following procedure may be employed. The rosin is melted with the plasticizer and filling materials are added by means of malaxating rolls and the like. Such material is then cut into blanks, heated on a steam table and assembled with the blanks of the cellulosic plastic material. The assembly is then pressed under elevated pressures and at elevated temperatures between matrices having the sound record therein. The sheets or films of cellulosic material adhere firmly to the core of the plasticized rosin.

By this invention sound records, which may be employed for reproducing and/or recording and which reproduce sounds of pure tone, may be made inexpensively. Furthermore the film or sheet of cellulosic plastic adheres firmly to the core of the plasticized rosin.

In order further to illustrate my invention, but without being limited thereto, the following specific example is given.

*Example*

40 850 parts of G H rosin are melted and to this are added

Parts by weight

45 Acetanilid----- 150  
Nigrosine----- 12.5

The acetanilid may be replaced in whole or in part with the plasticizer employed in making the cellulosic plastic.

50 After the ingredients have dissolved to form a homogeneous mass, there are thoroughly incorporated therein

Parts by weight

55 Lamp black----- 30  
Iron oxide----- 7½  
The lamp black and iron oxide are in finely pulverized form. The mass is then poured onto limed

concrete to cool, whereupon it solidifies into a glossy black solid. This is then broken up into small pieces and is then worked upon heated malaxating rolls during which time inert filling materials, such as a mixture of iron oxide, lamp black, barytes, china clay and cotton flock, in any desired amount may be added. During this time, if desired, shellac in amounts up to the amount of rosin present, may be added to the mass on the rolls.

The sheets formed on the rolls are cut into discs having a diameter of the finished record. Thereupon discs of cellulosic plastics are superposed upon the discs containing the rosin material. The cellulosic plastics may be of the following composition:

Parts by weight

|                            |     |
|----------------------------|-----|
| (A) Cellulose nitrate----- | 100 |
| Camphor-----               | 40  |

or

Parts by weight

|                            |     |
|----------------------------|-----|
| (B) Cellulose acetate----- | 100 |
| Diethyl phthalate-----     | 40  |

The assembly of the rosin composition core and the sheets or films of the cellulosic plastic is heated on steamed tables and pressed between sound matrices to produce the finished sound record.

It is to be understood that the foregoing detailed description is given merely by way of illustration and that many variations may be made therein without departing from the spirit of my invention.

Having described my invention, what I desire to secure by Letters Patent is:

1. A sound record having a reproducing surface contained in an outer layer made of a plastic composition having a basis of a derivative of cellulose, said record having an interior made of a composition having a basis of rosin, and containing the same plasticizer as is contained in the outer layer.

2. A sound record having a reproducing surface contained in an outer layer made of a plastic composition having a basis of cellulose acetate, said record having an interior made of a composition having a basis of rosin, and containing the same plasticizer as is contained in the outer layer.

3. A sound record having a reproducing surface contained in an outer layer made of a plastic composition having a basis of cellulose nitrate, said record having an interior made of a composition having a basis of rosin, and containing the same plasticizer as is contained in the outer layer.

GEORGE SCHNEIDER.

60

135

65

140

70

145

75

150